

## UNITED STATES PATENT OFFICE

1,989,101

PROCESS FOR IMPROVING ARTIFICIAL  
FIBERS OR FABRICS

Leon Lilienfeld, Vienna, Austria

No Drawing. Application May 29, 1929, Serial  
No. 367,150. In Austria June 18, 1928

8 Claims. (Cl. 8—20)

In application Serial No. 367,154 filed concurrently herewith is described a process wherein valuable properties are imparted to artificial silk (viscose silk, silk made by introducing viscose into  $H_2SO_4$  of 50% strength, or more, and known commercially as "Lilienfeld silk" "nitro silk", silk made by the cuprammonia process, and acetate silk), by treatment with a basic substance at a raised temperature, particularly with a solution of a caustic alkali or of an alkali sulphide. The improvement in the artificial silk is presumed to be dependent upon the raised temperature at which the treatment is conducted, a similar treatment at about ordinary temperature being incapable of producing the improvement.

I have now discovered that, contrary to what might be expected from the aforesaid specification, caustic alkali solutions of certain concentrations, namely containing not substantially below 36 per cent. of caustic alkali (calculated as NaOH) are capable of producing the aforesaid improvement at ordinary or moderate temperatures, but that the improvement attained at ordinary temperature, for example at 15°—25° C. or even at lower temperatures is at least equal to that attained by a similar treatment conducted at a high temperature with an alkali solution of equal strength.

My invention is based on this discovery, and consists in a process for improving artificial fibers by treating the material with a caustic alkali solution of at least 36 per cent. strength (calculated as NaOH) at a temperature not higher than 25° C.

If, for example, two samples of artificial silk in the form of fiber or fabric are treated respectively at 15° C. (according to the invention) and at 100° C. or higher, for example at 140° C., with a caustic soda solution of say 36, 40 or 50 per cent. strength, it will be found that in both cases the lustre and the feel have not appreciably suffered, the strength both in wet and dry state has not considerably diminished and the extensibility has increased.

The process according to the invention may be applied to artificial fibers in unstretched or only moderately stretched condition. The duration of the action of the strong alkali solution at ordinary temperature may be one minute or longer. The subsequent treatment of the material may consist in washing it directly with hot or cold water, or in introducing it directly into an acid bath, for example, into aqueous sulphuric acid of 10 to 20 per cent. strength and then washing.

Example 1.—Ordinary viscose silk in the form

of skeins is treated without stretching for one minute with a solution of caustic soda of 50 per cent. strength at 15° C. It is then removed from the caustic soda solution and treated with boiling water, then acidified in a sulphuric acid solution of 10 per cent. strength, washed and dried. It will then be found that the extensibility of this sample in the dry state has increased by 5 to 10 per cent., the lustre being excellent and the feel soft.

Example 2.—Mode of procedure as in Example 1, with the exception that, after being treated with the caustic soda solution, the artificial silk is introduced direct into sulphuric acid of 10 per cent. strength and then washed and dried.

Example 3.—Artificial silk made by the process described in my Patent No. 1,683,199 (namely by spinning viscose into a bath which has a plasticizing effect on the thread-like viscose stream during or immediately after its coagulation, for instance into sulphuric acid of not less than 55% strength) is immersed without stretching for one minute in a caustic soda solution of 50 per cent. strength at 15° C. and then finished as in Example 1 or 2. The material will be found to have an extensibility of 8 to 9 per cent. against 5 to 6 per cent. of the same silk in the untreated condition. Its feel is soft and its lustre unchanged.

The artificial silk prepared in accordance with said Patent 1,683,199 (later reissued as No. 18,170) is what is now commonly known as "Lilienfeld silk" and is characterized by high wet and dry strengths, i. e. by a dry tenacity of over 2 grams per denier (and sometimes 5 grams per denier or even more) and a wet tenacity of 1.5 grams per denier (and sometimes 2.5 grams per denier or even more). But that kind of artificial silk has an undesirably low extensibility. By treatment of this kind of artificial fiber, in accordance with the present invention, it is readily possible to increase the extensibility, without substantial injury to its other useful properties such as strength (wet and dry), lustre and soft silky feel (handle).

In the present process caustic alkali solutions of from 36 per cent. strength (calculated as NaOH) and more, up to solutions saturated at the temperature desired for the treatment may be used. Any temperature below 25° C. may be employed in the present process.

The expression "artificial fibers" as used in this specification and claims is intended to include all artificial fibers (such as artificial silk, artificial wool, artificial hair, artificial straw, in the form of spun material-threads yarns in skeins or cops, or in the form of warps, twisted yarn or the

5

10

15

20

25

30

35

40

45

50

55

like—and also in the form of fabrics) consisting of, or containing cellulosic bodies, such as cellulose, or cellulose hydrate or hydro-cellulose, or oxycellulose, or cellulose compounds, or cellulose derivatives of any kind.

Having thus described the nature of the said invention and the best means I know of carrying the same into practical effect, I claim:

- 5 1. A process of treating artificial fibrous textile material made from viscose by a regeneration process, which comprises contacting them with a caustic alkali solution of not substantially less than 36% strength (calculated as NaOH) at a temperature below 25° C., while allowing such 10 textile material to shrink, all without at any time treating such textile material with a viscose solution.
- 15 2. A process of treating artificial fibrous textile material made from viscose by a regeneration process, which comprises contacting them with a caustic alkali solution of not substantially less than 36% strength (calculated as NaOH) at a temperature below 25° C., while allowing such 20 textile material to shrink, and then washing such 25 treated textile material, and drying the same, all without at any time treating such textile material with a solution of a cellulose compound, containing an alkali metal trithiocarbonate.
- 25 3. In the treatment of textile materials made 30 from viscose by a regeneration process, the steps of contacting the same with a solution of caustic alkali of not substantially below 40% strength (calculated as NaOH), at a temperature not substantially above 25° C., and thereafter washing 35 out the alkali.
- 35 4. In the treatment of textile materials made 40 from viscose by a regeneration process, the steps of contacting the same with a solution of caustic alkali of not substantially below 50% strength, (calculated as NaOH), at a temperature not sub-

stantially above 25° C., and thereafter washing out the alkali.

5 5. In the treatment of artificial cellulosic threads regenerated from viscose, the steps of contacting the same with a caustic alkali solution of not substantially below 40% strength (calculated as NaOH), in a solvent liquid consisting of water, at a temperature not substantially above 25° C., and thereafter washing out the alkali.

10 6. A process for treating artificial textile fiber produced by spinning viscose into a bath which has a plasticizing effect on the thread-like viscose stream during or immediately after its coagulation, for instance into sulphuric acid of not 15 less than 55% strength, said fiber having a dry tenacity exceeding 2 grams per denier, which comprises contacting them with a caustic alkali solution of not less than 36% strength (calculated as NaOH), in a liquid solvent consisting of water, 20 at a temperature below 25° C., in the absence of a cellulose compound containing alkali metal tri-thiocarbonate.

25 7. A process as in claim 6, wherein the artificial fibers are treated with the caustic alkali solution while in an unstretched condition.

30 8. A process for treating artificial textile fiber produced by spinning viscose into a bath which has a plasticizing effect on the thread-like viscose stream during or immediately after its coagulation, for instance into sulphuric acid of not less than 55% strength, said artificial fiber having a dry tenacity exceeding 2 grams per denier, which comprises contacting the same with a 35 caustic alkali solution of not less than 36% strength (calculated as NaOH) at a temperature below 25° C., then washing the treated artificial fiber, and drying the same.

LEON LILIENFELD. 40